# EUROPEAN PATENT SPECIFICATION

(11) **EP 0 156 482 B1**
(45) Date of publication and mention of the grant of the patent: **24.05.1989**
(21) Application number: 85300957.9
(22) Date of filing: 13.02.1985
(51) Int. Cl.: C22C 19/07, H01F 1/04

(54) **Sm2Co17 alloys suitable for use as permanent magnets**
Sm2 Co17-Legierungen, die für Dauermagnete anwendbar sind
Alliages Sm2 CO17 utilisables comme aimants permanents

(30) Priority: 13.02.1984 GB 8403752; 13.02.1984 GB 8403751
(43) Date of publication of application: 02.10.1985
(73) Proprietor: Sherritt Gordon Limited, Toronto, Ontario (CA)
(72) Inventor: Wysierkierski, Andrew G., Fort Saskatchewan Alberta (CA); Fraser, Robert W., Fort Saskatchewan Alberta (CA); Clegg, Maurice A., Fort Saskatchewan Alberta (CA)
(74) Representative: Lambert, Hugh Richmond

(56) References cited:
- DE-A- 2 727 243
- DE-A- 2 944 031
- GB-A- 2 021 147
- GB-A- 2 089 371
- US-A- 4 172 717
- US-A- 4 221 613

## Description

This invention relates to Sm₂Co₁₇ alloys suitable for use as permanent magnets.

The advantages of rare earth cobalt alloy magnets are now well known. Such magnets are specially suitable for use in electric motors, such as DC servomotors. It is also known that SM₂CO₁₇ alloys have potential advantages for use as permanent magnets over SmCo₅ alloys⁽¹⁾. For example, DC motors using Sm₂Co₁₇ alloy magnets have lower weight and inertia and increased torque and acceleration compared to the use of SmCoₛ alloy magnets.

Various attempts have been made to provide Sm₂Co₁₇ alloys which can form permanent magnets having a high energy product (BH)max and a high intrinsic coercivity ₁Hc. Typical prior art is shown for example in United States patent No. 4,172,717 issued October 30, 1979 to Tokunaga et al⁽²⁾, United States patent No. 4,213,803 issued July 22, 1980 to Yoneyama et al⁽³⁾, United States patent No. 4,221,613 issued September 9, 1980 to Imaizumi et al⁽⁴⁾ and United States patent No. 4,375,996 issued March 8, 1983 to Tawara et al⁽⁵⁾. Other prior art is shown in the published literature ^{(6, 7, 8, 9, 10)}.

As disclosed in the above-mentioned prior art, SM₂CO₁₇ alloys are known which can form magnets having an energy product (BH)ₘₐₓ in the range of 22 to 30 MGOe and an intrinsic coercivity ₁H_{c} in the range of 5.8 to 6.3 kOe^{(6, 7)}. Later developments have resulted in the production of Sm₂Co₁₇ alloys which can produce magnets with higher coercivity, but this advantage has been offset by loss in energy product. For example, one Sm₂CO₁₇ alloy is now known which can produce magnets having an energy product (BH)ₘₐₓ of 26 MGOe and an intrinsic coercivity ₁H_{c} of 15.0 kOe⁽⁷⁾. Another Sm₂CO₁₇ alloy now known has an energy product (BH)ₘₐₓ of 27 MGOe and an intrinsic coercivity ᵢH_{c} of 10.0 kOe, see United States Patent No. 4,375,996 mentioned above⁽⁵⁾.

Additionally, GB-A-2,089,371 discloses Sm₂CO₁₇ containing resin- or metal-bonded permanent magnets obtained by first heat treating a bulk ingot to obtain magnetic properties, crushing and grinding the ingot to particles not larger than 50 um, and compacting these particles with a binder in a magnetic field. A very wide range of alloys is disclosed, namely alloys containing
21-28% Sm
3-10% Cu
14-35% Fe
0.5-5% Zr, Ti, Hf, Ta, Nb, Va. In such alloys, relatively low magnetic properties are obtained, viz. energy products (BH)ₘₐₓ in the range 3.8 to 17 MGOe and residual induction values Bᵣ in the range 6.8 to 8.68 kG.

In GB-A-2,021,147 R₂C_{O17} type permanent magnet alloys, where R is a rare earth metal e.g. samarium, are disclosed to which hafnium is added to provide alloys with high coercive force even when the Cu content is low and the Fe content is high. Disclosed values for the maximum energy product, BHₘₐₓ, range from 26 to 29.5 MGOe, coercive force, bHc, from 7.4 to 7.5 kOe, and magnetic remanence, Br, from 10.5 to 11.0 KG. Such values are obtained in R₂CO₁₇ type alloys in which the atomic ratios of the rare earth metal R (which is preferably Sm, but may alternatively be one or more other rare earth metals, including mixtures, for example, in which the Sm is at least partially replaced by praseodymium Pr), Cu, Fe and Hf (or other selected transition metal) are represented by the formula

where
R=inter alia Sm,
0<u<0.2
0.1 <v<0.6
0.005<w<0.05
6.5<z<8.8 and which may additionally contain an amount x of one or more of Ti, V Cr, Zr, Nb, Mo, Ta, W, Ru, Rh, Pd, Ag, Cd, Pt and Au where 0.003<x<0.05.

It is also known that, because of different magnetic hardening mechanisms, Sm₂CO₁₇ alloys are harder to magnetize from an unmagnetized state than SmCo₅ alloys. For example, in the construction of electric motors, it is the preferred practice to construct the field or stator assembly with unmagnetized magnets, and then magnetize the finished assembly as a single unit. This preferred industrial practice imposes an upper limit of about 25 kOe on the intensity of the magnetizing field which can be applied to the unmagnetized magnets of a typical assembly. Thus, in order to be useful in practice, an unmagnetized magnet must be capable of attaining its specified properties in a magnetizing field of 25 kOe. To date, it has not been possible to achieve this requirement with Sm₂Co₁₇ alloys with an energy product greater than 30 MGOe⁽⁶⁾.

Thus, although it is acknowledged that Sm₂Co₁₇ alloys have potential advantages over other rare earth/transition metal alloys such as SmCo₅ alloys, Sm₂CO₁₇ alloys have not yet become practically useful because improved coercivity has only been obtainable at the expense of energy product and also because such alloys have not been capable of attaining their specified properties in a magnetizing field up to about 25 kOe.

More specifically, the prior art has not appreciated the precise nature of the hardening mechanism in Sm_{z}COᵢ₇ magnets, and the effect thereof on the magnetic properties of the alloy, and the need to exercise precise control over the amount of samarium and zirconium in the alloy in order to obtain superior magnetic properties, inter alia, energy products BHₘₐₓ of at least 30 MGOe and remanent induction values of at least 11.5 kG.

In accordance with the present invention, Sm₂Co₁₇ alloys are provided which are suitable for use in the manufacture of permanent magnets of high energy product and high coercivity, such alloys consisting of, on a weight basis and apart from impurities:
(a) an amount of samarium that is equal to from 22.5 to 23.5% of the alloy plus an additional percentage that is equal to from 4 to 9 times the amount of oxygen;
(b) from 20.0 to 25.0% Fe;
(c) from 3.0 to 5.0% Cu;
(d) an amount of zirconium that is equal to from 1.4 to 2.0% of the alloy plus an additional percentage that is equal to from 5 to 10 times the amount of carbon;
(e) not more than 0.6% oxygen;
(f) not more than 0.1% carbon; and
(g) balance cobalt; said alloy having a crystallographic structure comprising cells of 2-17 Sm-Co rhombohedral phase surrounded by a continuous network of the 1-5 Sm-Co hexagonal phase, such structure being obtainable by:
   (i) sintering an alloy of the required chemical composition at a temperature at which the alloy consists in the form of a solid/liquids mixture, the solid phase consisting essentially of solid grains of 2-17 Sm-Co, and the surrounding liquid phase comprising a CuSm phase and a Zr-rich phase;
   (ii) cooling the sintered alloy slowly to a solid solution treatment temperature marginally below the solid+liquid/solid transformation temperature of the alloy, thereby to form a homogeneous solid solution of said CuSm and Zr-rich phases in the 2-17 Sm-Co phase;
   (iii) holding the alloy at said solid solution treatment temperature to promote the formation of said solid solution;
   (iv) quenching the alloy from said solution treatment temperature to room temperature;
   (v) reheating the alloy to a first aging temperature at which the solid solution transforms into a structure comprising a network of the 1-5 Sm-Co phase within a 2-17 Sm-Co matrix;
   (vi) cooling the alloy slowly to a second aging temperature to cause regions of the 2-17 Sm-Co phase to nucleate coherently within the 1-5 Sm-Co phase network and thereby to create lattice strain therein; and
   (vii) recooling the alloy to room temperature.

Within the above alloy composition the amounts of oxygen and carbon are "incidental", that is to say no attempt is made deliberately to incorporate oxygen and carbon into the alloy, the amounts of oxygen and carbon appearing in the alloy as a matter of course, and which are therefore inevitable in such compositions unless elaborate precautions are taken to exclude them. Thus it is a feature of the invention that the inevitability of such incidental amounts of oxygen and carbon in the alloy composition is recognised, and the invention recognises that it is necessary that an additional amount of Sm should be provided to compensate for the oxygen content and that an additional amount of Zr should be provided to compensate for the carbon content. Preferably, the additional amount of Sm is 6.265 times the oxygen content, and the additional amount of Zr is preferably 7.595 times the carbon content. The remainder of the alloy content is cobalt.

The function of the first specified amount of samarium, hereinafter referred to as the "effective samarium" is to develop the desired cryatallographic structure consisting of cells of the 2-17 Sm-Co rhombohedral phase surrounded by a continuous network of the 1-5 Sm-Co hexagonal phase⁽¹¹, ^{12, 13)}. It is necessary that the 1-5 network be continuous to develop the desired second quadrant loop squareness, that is to say a maximum value of H_{K}, and that is dependent upon the "effective samarium" present. Sufficient samarium must be present for this purpose but too much samarium results in the breakdown of the 2-17 rhombohedral phase and loss of remanent induction Bᵣ. The function of the "effective samarium" present is therefore to develop the 2-17 Sm-Co rhombohedral phase having high remanent induction B, and to develop a complete 1-5 Sm-Co hexagonal phase network to develop the coercivity or magnetic hardening. Too little samarium results in an incomplete 1-5 Sm-Co network and incomplete hardening, that is to say a low H_{K}, and too much samarium results in a breakdown of the 2-17 Sm-Co phase and loss of remanent induction B, and energy product (BH)_{maX}. Precise control of the "effective samarium" content is necessary to obtain optimum properties and this can be achieved by the present invention.

The function of the first amount of zirconium, hereinafter likewise referred to as "effective zirconium" is to facilitate the dissolution of all the desired constituents into one single phase solid solution in the solution heat treatment stage of the processing. Only when this is achieved is it possible to establish complete homogeneity as the necessary starting point to develop in the subsequent aging heat treatment the desired structure consisting of 2-17 Sm-Co cells surrounded by a continuous network of the 1-5 Sm-Co boundary phase. The presence of zirconium distorts the Sm-Co lattice so as to reduce the c/a ratio of the hexagonal unit cell(¹⁴) and this facilitates the accommodation of the desired elements in single phase solid solution during the solution heat treatment at 1140-1170°C. At elevated temperatures the 2-17 Sm-Co composition has a hexagonal crystal lattice but at room temperature it transforms to a rhombohedral crystal lattice. These two crystal systems are closely related and the rhombohedral lattice can be regarded as an imperfect hexagonal lattice containing stacking faults. The desired equilibrium structure at room temperature consists of cells of the 2-17 Sm-Co rhombohedral phase surrounded by a continuous network of the 1-5 Sm-Co hexagonal phase. It has also been observed that for a fixed copper content the coercivity increases with the zirconium content. Thus to achieve the objective of easier magnetization it is necessary to keep the zirconium content to a minimum commensurate with the above stated requirements regarding the single phase solid solution. The necessary precise control of the "effective zirconium" content can be achieved by the present invention.

By using an SM2CO1, alloy in accordance with the invention, it is possible to produce a permanent magnet which attains its specified properties in a magnetizing field of about 25 kOe, has an energy product (BH)ₘₐₓ of at least 30 MGOe and has a satisfactory coercivity H, of 14 to 16 kOe. A magnet in accordance with the present invention can also have a satisfactory remanent induction Bᵣ of at least about 11.5 kG, and a better loop squareness in the second quadrant, i.e. H_{K} of approximately 9.0 kOe.

A preferred alloy in accordance with the invention contains:
23.0% Sm as the first or effective amount,
22.0% Fe,
4.6% Cu,
1.5% Zr as the first or effective amount,
minor amounts of oxygen and carbon, i.e. not greater than 0.6% and 0.1% respectively,
additional amounts of Sm and Zr as specified above, viz. from 4 to 9 times the oxygen content for samarium, preferably 6.265 times, and from 5 to 10 times the carbon content for zirconium, preferably 7.595 times,
and the balance being cobalt.

The invention is at least partly based upon the realization that it is possible to compensate for small traces of carbon present in many of the elements that are used in the production of the alloy and which have an adverse effect on the magnetic properties of the alloy. In accordance with the invention, compensation is made for the carbon content by providing an additional amount of zirconium as specified above.

The additional zirconium may be incorporated in the alloy by adding zirconium in the form of a master alloy to an Sm₂CO₁₇ base alloy at a convenient stage in the processing, for example prior to compacting and sintering the alloy powder. The master alloy may be of a simple form such as ferrozirconium, which is a low melting point (about 935°C) eutectic containing 83% Zr and 17% Fe by weight. Ferrozirconium may be successfully used when only a small additional amount of zirconium is required. In other words, only up to about 2% ferrozirconium by weight should be added.

If a larger additional amount of zirconium has to be added, it is preferable to utilize a master alloy with the same composition as the base alloy with the exception that the master alloy should contain a larger amount of zirconium, for example from about 5 to 10% by weight, the increase in the zirconium content being achieved at the expense of the cobalt content.

The following table illustrates the compensation of zirconium content for carbon present and the optimum zirconium level at about 1.5%.

The present invention is also at least partly based on the realization that it is possible to compensate for the small traces of oxygen which are picked up by the alloy during its manufacture and which have an adverse effect on the magnetic properties of the alloy. In accordance with the invention, the small traces of oxygen are compensated for by addition of an additional amount of samarium as specified above. The amount of oxygen in the final product can be estimated from the oxygen content of the starting material or more preferably determined by analyzing a sample product.

The samarium addition may be accomplished by adding a samarium rich alloy to a Sm₂Co₁₇ base alloy at a convenient stage in the processing, for example prior to compacting and sintering the alloy powder. It is not practicable to add elemental samarium because of its high rate of oxidation. The samarium rich alloy preferably has the same composition as the base alloy except that the samarium content would be about 1 to 3% higher than in the base alloy, the higher samarium content being achieved at the expense of the cobalt content. A simple binary master alloy (such as 60% Sm, 40% Co) can also be used to add Sm.

The following table illustrates the compensation of samarium content for oxygen present and the optimum effective samarium in the range 22.523.5%.

By adding additional zirconium and samarium to compensate for the inevitable presence of small traces of carbon and oxygen in the alloy, it has been found to be possible to define more precisely the alloy composition in order to produce the preferred magnetic properties.

Thus, the preferred samarium range is 22.5 to 23.5% with the preferred samarium value being 23.0% Sm. This is the effective amount, as compared to the additional amount provided as specified to compensate for oxygen content. The range of effective samarium content is considerably narrower than has been specified in the prior art.

The effective zirconium range has been specified to be from 1.4 to 2.0% with the preferred value being 1.5%. Thus, with the present invention, it has been possible to specify a zirconium range which is considerably narrower than that taught by the prior art.

It has also been found possible to optimize the iron and copper contents. The composition limits of iron, copper and zirconium are interrelated and each can critically affect the existence of the single phase structure. It is known that the addition of iron to the 2-17 Sm-Co system increases the remanent induction provided that the structure can be maintained as a single 2-17 Sm-Co phase. If the optimum iron content is exceeded the alloy breaks down into an Fe-rich eutectoid structure having lower remanent induction, It has been observed that the copper content acts to increase the coercivity or magnetic hardness of the alloy. It is believed that copper concentrates in the 1-5 Sm-Co phase network and enhances the coherent nucleation of regions of 2-17 Sm-Co phase within the 1-5 Sm-Co phase network during cooling from the aging temperature, thereby creating lattice strain and magnetic hardness or coercivity⁽¹⁵⁾.

The iron content has been specified to be 20.0 to 25.0%, preferably 22.0%, and the copper content has been specified to be 3.0 to 5.0%, preferably 4.6%. The iron content has also been defined within a much narrower range than has been taught by the prior art. Similar remarks apply to the copper content. As previously indicated, cobalt forms the balance of the composition.

An Sm₂CO₁₇ alloy in accordance with the invention is preferably made in the following manner. The alloy of the desired composition was produced by pulverizing melted and cast alloy into particles of 3-8 11m size. Small additions of ferrozirconium and a samarium rich alloy of similar composition to the parent alloy were then blended in to compensate for the deleterious effects of the trace amounts of carbon and oxygen present according to the present invention. The blended powders were aligned in a die under a transverse magnetic field of 12 kOe and compacted under a pressure of 60 kpsi. The green compact was sintered in hydrogen at 1150°C for 30 min. The atmosphere was then changed to argon and the compact was heated to 1205°C at a rate of 4-5°C/min, held at 1205°C for 10 min and then cooled to 1160°C at 2°C/min. The sample was then solution treated at 1140-1160°C for 2 hours, quenched from 1140-800°C at 10°C/s and air cooled from 800°C to room temperature. It was then reheated to 845±5°C and held for 20 hours, cooled at about 2°C/min from 845°C to about 600°C and at about 1°C/min from about 600°C to 410°C, held at 410°C for 10 hours and cooled to room temperature.

An Sm₂CO₁₇ alloy having the previously mentioned preferred composition in accordance with the invention and produced in the above described manner achieved the following properties:

The advantage of the invention can readily be seen from the above Table.

It has also been found that praseodymium can be substituted in part for samarium in the alloy of the present invention without decreasing the aforementioned desirable properties. To preserve the required 2-17 Sm-Co rhombohedral crystal structure the substitution of praseodymium must be made on an atomic basis, that is to say since praseodymium has a lower atomic weight than samarium, on a weight percent basis less praseodymium will be required in the alloy than the weight percent of samarium replaced. In the example illustrated below it was found that whereas optimum properties were obtained with 23.0% effective samarium in the standard alloy, when a combination of samarium and praseodymium was used the optimum properties were obtained with an effective amount of 22.5% (Sm+Pr), comprising 20.0% Sm+2.5% Pr. Furthermore, in calculating the effective amount of praseodymium present with respect to that amount which has been rendered ineffective by combination with oxygen, account must be taken of the molecular weight of the praseodymium oxide and the correction factor of 6.265 times the oxygen content for samarium must be changed to 5.871 for the praseodymium added. Also as is described more fully in copending European Application EP-A-0 156483 filed simultaneously herewith and claiming priority from U.K. 8403751 and to which reference should be made, in the production of high strength 2-17 Sm-Co permanent magnets from the alloys of the present composition the selection of a solution treatment temperature which is marginally below the liquid plus solid phase transformation temperature for the specific alloy composition is important. In the case where praseodymium has been partially substituted for samarium care must be taken since the liquid plus solid phase transformation temperature will be lower than that of the standard samarium alloy by an amount depending on the level of praseodymium substituted. The following example illustrates the partial replacement of samarium by praseodymium. An alloy containing 20.3% Sm and 2.17% Pr as effective amounts was prepared as described earlier with the exception that the solution treatment step was carried out in the range 1130-1150°C. The following properties were obtained and are compared with those of a similar alloy containing only samarium as the rare earth element.

It has also been found that other group IVB or VB transition elements may be substituted full or in part for zirconium in the alloy of the present invention. Since the function of the group IVB or VB transition element is to reduce the c/a ratio of the 2-17 Sm-Co hexagonal unit cell, the replacement of zirconium by other elements must be made on an atomic basis. Furthermore in calculating the effective amount of the transition metal present with respect to that amount rendered ineffective by combination with carbon, account must be taken of the molecular weight of the transition metal carbide and the correction factor of 7.595 times the carbon content of the alloy must be adjusted accordingly. For example, in the case of hafnium the correction factor would be 14.862 times the carbon content of the alloy. Moreover, and as is pointed out in said copending application, in the process for the production of high strength 2-17 Sm-Co permanent magnets from these alloys, the aging temperature is critically dependent upon the zirconium content. Thus where other group IVB or VB transition elements are substituted for zirconium in the alloy the optimum aging temperature and time may be different from those referred to above where Zr is the sole group IVB or VB element. The following example illustrates the substitution of hafnium for zirconium in an alloy of the present invention. An alloy was prepared as described earlier for the standard alloy except that zirconium as an effective amount was replaced by hafnium as an effective amount. In calculating the additional amount of hafnium required to arriveat the effective amount the carbon content of the alloy was multiplied by the factor 14.862. The alloy was processed as described earlier for the standard alloy with the exception that after quenching from the solution temperature to room temperature the alloy was reheated to an aging temperature of 845±5°C and held there for 24 hours.

The following table illustrates the replacement of zirconium by hafnium as an effective amount.

The invention thus also provides an Sm2Co» alloy permanent magnet containing also iron, copper and zirconium or similar group IVB or VB transition metals, said alloy containing: an effective amount of samarium, in addition to that samarium combined with oxygen, such that after the aging stage of the process the crystal structure of the alloy consists of the single phase 2-17 Sm-Co rhombohedral structure containing a continuous network of the 1-5 Sm-Co phase, an effective amount of zirconium, in addition to that zirconium combined with carbon, such that during the solution heat treatment stage of the process the 2-17 Sm-Co crystal lattice is distorted to facilitate the dissolution of all the constituents of said alloy into a uniform single phase solid solution, an amount of iron being as high as possible to maximize the remanent induction of said alloy whilst still maintaining the single phase 2-17 Sm-Co uniform solid solution in the solution heat treatment stage of the process, an amount of copper such that during the cooling stage from the aging temperature the coherent nucleation of 2-17 Sm-Co phase within the 1-5 Sm-Co phase network is enhanced to produce lattice strain and coercivity, it being understood that both zirconium and copper levels must be controlled to permit the iron level to be optimized whilst still maintaining a uniform solid solution in the solution heat treatment stage.

The optimization of composition must be based on the requirement that all the alloying elements are first put into a uniform solid solution. In the studies of composition variations in Fe, Cu and Zr it was found that the optimum effective samarium content remained constant at 23±0.5%. However, it was found that the effective samarium content can be partly replaced by praseodymium with the added observation that slightly less (Sm+Pr) is required for optimum properties. From an economic point of view this could be an attractive alternative.

In more detail the alloys described above can be produced by means of a process in which a sintering step is followed by a solution treatment step, with the alloy being cooled from a sintering temperature to a solid solution treatment temperature in a controlled manner such that all the alloying elements are put into uniform solid solution.

It has been found that such controlled cooling from the sintering temperature to the solid solution treatment temperature enables all the constituents to be dissolved into a homogeneous solid solution and enables improved magnetic properties to be obtained in an SM₂CO₁₇ alloy. For example, it is possible for the alloy to have a relatively high iron content (to provide high remanent induction) without the 2-17 Sm-Co phase being rendered unstable, and to have a relatively high samarium content to provide good second quadrant loop squareness. With prior art processes, it was found that the presence of a high iron content causes the required 2-17 Sm-Co rhombohedral phase to become unstable, with resultant transformation to iron-rich phases and consequent deterioration of magnetic properties, especially remanent induction.

By using such a process it is possible to produce a permanent magnet which attains its specified properties in a magnetizing field of about 25 kOe, has an energy product (BH)ₘₐₓ of at least 30 MGOe and has a satisfactory intrinsic coercivity ᵢH_{c} of 14-16 kOe. A magnet in accordance with the present invention can also have a satisfactory remanent induction Bᵣ of at least about 11.5 kG and a better loop squareness in the second quadrant, i.e. H_{K} of approximately 9.0 kOe.

It has been found that the initial alloy body should be sintered at the highest possible temperature in the liquid+solid region to achieve full density and high remanent induction. The sintering temperature may be at least about 1200°C at at least the end of the sintering step. The sintering temperature should be such that the alloy consists at that temperature of a mixture of liquid and solid phases to promote rapid sintering. The predominant solid phase consists of 2-17 Sm-Co grains, with these being surrounded by a liquid phase comprising a CuSm phase which also contains a small amount of a Zr-rich phase.

The sintering process may be carried out in an inert atmosphere such as argon, or in hydrogen or in a vacuum, or in a combination of these. In the case of sintering solely in an atmosphere of argon the possibility exists that some argon may be trapped in pores within the sintered alloy. This undesirable occurrence can be minimized by sintering initially at a somewhat lower temperature in a vacuum so as to decrease the porosity and then increasing the temperature in an argon atmosphere to achieve full density. Similarly it is not practical to sinter entirely in a vacuum as excessive loss of samarium would result and the preferred procedure would be to sinter initially at a lower temperature in a vacuum and then change to an argon atmosphere before raising the temperature to the desired higher level. Alternatively the alloy may be sintered initially in an atmosphere of hydrogen at a somewhat lower temperature, for example 1150°C for 30 min, to close the internal porosity, followed by heating to the range of 12001215°C in an atmosphere of argon and holding at that temperature for 10 min.

In accordance with the invention, the sintered alloy body is cooled in a controlled manner from the sintering temperature to a solid solution treatment temperature to ensure homogeneous equilibrium dissolution of the CuSm and Zr-rich phases into solid solution in the stable 2-17 Sm-Co phase. A relatively high iron content renders such dissolution more difficult to achieve since the high iron content reduces the temperature range within which the stable 2-17 Sm-Co solid phase exists as a single phase. However, the controlled cooling from the sintering temperature to the solution treatment temperature in accordance with the invention enables this problem to be overcome.

If a sintered alloy body with relatively higher iron content is cooled too rapidly from the sintering temperature to the solid solution treatment temperature, the CuSm and Zr-rich phases remain concentrated at the grain boundaries. The localized high concentration of samarium results in transformation of the 2-17 Sm-Co phase to an Fe-rich phase with lower remanent induction. Also, in the same grain boundary region, zirconium may be rejected from solid solution, with a resultant adverse effect on loop squareness. The possibility of occurrence of such undesired effects is significantly reduced by slow cooling from 1170°C to the solid solution treatment temperature in accordance with the present invention.

After slow cooling to the solid solution treatment temperature, which is marginally below the solid+liquid/solid phase transformation temperature for the alloy composition and which may for example be from about 1140 to about 1150°C, the alloy body is maintained at this temperature for a period of time (for example about 2 hours) to improve the dissolution of the alloying elements and to remove any structural faults by annealing. The alloy body is then quenched from the solid solution treatment temperature to a temperature below 800°C at a rate of about 10°C/s, and thereafter to room temperature. In our co-pending application it is disclosed that optionally part of the samarium may be replaced by praseodymium. In this case the solid+liquid/solid phase transformation temperature will be lower and the solid solution treatment temperature must be lower, in the range 1120-1145°C.

The alloy body is then aged to develop the 1-5 Sm-Co phase network. The aging temperature will be generally in the range of 800-860°C but must be precisely chosen depending on the composition, in particular on the zirconium content. A preferred aging temperature in the present invention is 845±5°Cfor 20 hours.

After the aging step, it is necessary to cool the alloy body in a controlled manner to effect the required magnetic hardening, that is to say achieve the required intrinsic coercivity and good loop squareness. Such controlled cooling may be from the aging temperature to about 600°C at a rate preferably about 2°C/min and from about 600°C to the secondary aging temperature in the region of 400°C at about 1°C/min. A preferred secondary aging treatment in the present invention is 410°C for 10 hours. The alloy body is then cooled to room temperature.

It is postulated that during cooling from the first aging temperature and during holding at the second aging temperature regions of 2-17 Sm-Co phase nucleate coherently within the 1-5 Sm-Co phase network thereby creating lattice strain and magnetic hardening(¹⁶). When magnetically hardened, the 1-5 Sm-Co phase network serves as a barrier to magnetic domain wall motion and creates the required intrinsic coercivity and good second quadrant loop squareness.

An alloy body in accordance with one embodiment of the invention was produced in preliminary form with the following composition by weight: 22.7% effective Sm, 22.0% Fe, 4.6% Cu, 1.5% effective Zr, and balance cobalt. The alloy body was sintered for 30 min in hydrogen at 1150°C, and for 10 min in argon at 1205°C. The sintered alloy body was then cooled to 1150°C at a rate of 2°C/min.

The alloy body was then subjected to solid solution treatment at a temperature of 1140 to 1150°C for 2 hours. After the solid solution treatment, the alloy body was quenched to room temperature. A micrograph showed that a uniform single phase solid solution structure was achieved.

The alloy body was then aged by reheating to 815°C and maintained at that temperature for 20 hours, then the alloy body was cooled to 600°C at a rate of 2°C/min and from 600° to 410°C at a rate of 1°C/min, held at 410°C for 10 hours and then cooled to room temperature. A micrograph was taken and showed a uniform structure of 2-17 Sm-Co grains.

Another alloy body having the same composition as the previous alloy body was prepared and subjected to the same treatment as the previous alloy body, except that cooling from the sintering temperature to the solid solution treatment temperature was effected at a rapid rate of 10°C/s. The alloy was then reheated to 815°C and aged as described above. A micrograph was taken and showed large grains constituting the 2-17 Sm-Co phase, with a CuSm black phase and a Zr-rich white phase being seen in the grain boundary area.

The alloy bodies were then magnetized in a magnetizing field of 25 kOe and the resulting magnetic properties were measured, as shown in the following Table.

The superior magnetic properties of the alloy body which was subjected to slow cooling from the sintering temperature to the solid solution treatment temperature in accordance with the invention are readily apparent.

It was found that in the sintering process it is advantageous to sinter first in an atmosphere of hydrogen followed by a further period in an atmosphere of argon. For example, a preferred sintering process is to sinter for 30 min in hydrogen at 1150°C, change the furnace atmosphere to argon, increase the temperature at 4-5°C/min to 1205°C and maintain this temperature for 10 min. It was observed that during the first sintering treatment the density of the product increases by pore closure with entrapment of some hydrogen. In the second sintering treatment in argon the internal hydrogen is removed by diffusion and the remaining pores are closed to full density. No argon entrapment occurs during the second sintering treatment as the external porosity has been sufficiently closed by the initial sintering treatment, and no hydrogen remains in the alloy as the final sintering treatment is carried out in argon. If the entire sintering treatment is carried out in argon, some argon is trapped within the internal porosity and results in residual porosity, lower density and lower remanence (Bᵣ) in the finished magnet.

To achieve improved magnetic properties, e.g. higher energy product, systematic increases were made in the Fe content and it was found that it was necessary to adjust the other elements accordingly and to adjust the temperature and time of the solution heat treatment to achieve the basic requirement of putting all the alloying elements into uniform solid solution. For example, to increase the Fe content from 15% to 22% it was also necessary to reduce the Cu content from 6.0% to 4.6% and the effective Zr content from 2.5% to 1.5% and to modify the solution heat treatment from one hour at 1180°C to a controlled cooling procedure from the sintering temperature of 1205°C to the solution heat treatment temperature which is marginally below the solid+liquid/solid phase transformation temperature. This temperature is dependent upon the precise composition and may be determined metallographically. The major influence on this transformation temperature is that observed for iron, for example, for alloys containing 15% Fe the transformation temperature was determined to be 1180°C, for 17% Fe, 1170°C and for 22% Fe, 1150°C, i.e. there is approximately 4°C decrease in transformation temperature for 1 % Fe increase in the range studied to date.

Following solution treatment, the alloy is quenched to room temperature and reheated to the aging temperature in the range of 800-860°C for up to 20 hours. In this aging treatment the 2-17 Sm-Co solid solution transforms into a duplex structure consisting of a continuous network of 1-5 Sm-Co phase within the 2-17 Sm-Co matrix. We have found that this broad range of 800-860°C for the aging temperature is not acceptable and that the aging temperature must be precisely determined with respect to the zirconium content. For example, the optimum aging temperature was found to be 815±5°C for an effective zirconium content of 2.0-2.5%. For lower zirconium contents the aging temperature must be raised. For example, the optimum aging temperature was found to be 845±5°C for an effective zirconium content of 1.42.0%. It was found that a minimum time of about 20 hours is required at the aging temperature to form the required 1-5 Sm-Co phase network to develop the desired coercivity. Shorter times, i.e. 10 and 15 hours, result in lower coercivities and longer times, i.e. 30 hours, do not produce any further improvements. To develop the required coercivity and loop squareness (H_{K}) it is necessary to have a continuous network of the 1-5 Sm-Co phase. This requires sufficient samarium to be present and we have found 22.5-23.5% effective samarium to be a preferred amount.

In this aging treatment, it has been observed that the nature of the structural change taking place is critically dependent upon the temperature at which the aging process is started, that is to say the same result cannot be obtained by using a higher temperature for a shorter time or vice versa. This behaviour is typical of a spinoidal decomposition as distinct from a nucleation and growth reaction.

Following this primary aging treatment at about 800-860°C the specimen must be cooled to the secondary aging temperature in the range 400-425°C at a critical rate. The preferred cooling rate is about 2°C/min from the aging temperature to about 600°C and about 1°C/min from about 600°C to the secondary aging temperature. Small variations to the above do not appear to have a deleterious effect, however cooling rapidly such as >2°C/min or very slowly such as <0.5°C/min resulted in inferior magnetic properties. It is postulated that during this critical cooling step regions of 2-17 Sm-Co phase nucleate coherently within the 1-5 Sm-Co phase network, thereby causing lattice strain and creating the coer_{C}i_{V}ity(¹⁶¹. This transformation is enhanced by the presence of copper in the 1-5 Sm-Co phase. From this model it is understood that faster cooling rates do not permit regions of the 1-5 Sm-Co phase to transform to the 2-17 Sm-Co phase, and slower cooling rates allow incoherent nucleation to take place without lattice strain.

In the 1-5 Sm-Co system containing copper, the aging process to develop coercivity shows an optimum temperature in the range of 400―450°C⁽¹⁶⁾. It was found that in 2-17 Sm-Co magnets in accordance with the invention in which coercivity and loop squareness (H_{K}) are being developed by aging the 1-5 Sm-Co phase network containing copper, the same effect applies. The optimum aging temperature was found to be 410-4.15°C. With an aging temperature of 400°C for 10 hours a lower loop squareness (H_{K}) was obtained as was also the case at 422°C, as shown below.

It has been found that an aging treatment of 10 hours at 410-415°C is effective. It is also believed that the optimum secondary aging temperature is dependent upon the copper content.

It was found that the final cooling step to room temperature after aging at 400-425°C is not critical.

The present invention also provides a process for producing an Sm₂Co₁₇ alloy permanent magnet, containing also iron, copper and zirconium or a similar group IVB or VB transition metal, the process comprising: providing said alloy in a preliminary form, sintering said alloy at an elevated temperature to achieve a high density which results in a high remanence, selecting a solution treatment temperature which is marginally below the liquid+solid/solid phase transformation temperature for the preferred composition of said alloy, cooling the alloy from the elevated sintering temperature to the solution treatment temperature in a controlled manner such that all the alloy constituents are put into a uniform solid solution, holding at the solid solution treatment temperature, quenching the alloy to room temperature, reheating the alloy to the aging temperature, which is critically dependent on the composition of said alloy, particularly the zirconium content, and holding for sufficient time for the 2-17 Sm-Co solid solution to transform into a structure consisting of a continuous network of the 1-5 Sm-Co phase within the 2-17 Sm-Co matrix, cooling said alloy to the secondary aging temperature at a critical rate and holding at that temperature for a specified time such that regions of 2-17 Sm-Co phase nucleate coherently within the 1-5 Sm-Co phase network thereby creating lattice strain which results in high coercivity and good loop squareness, and cooling said alloy from the secondary aging temperature to room temperature.

The following comments in connection with the invention are also appropriate:
1. A high sintering temperature develops a high density and this results in ultimately a high remanence. To minimize distortion a two stage process is preferred; 30 min in hydrogen at 1150°Cfollowed by heating in argon at 4-5°C/min to 1205°C and holding at this temperature for 10 min.
2. A high iron content is desirable to increase the remanence and energy product but the copper and zirconium contents must be reduced as the iron is increased to maintain the uniform 2-17 Sm-Co solid solution. Iron has the most marked effect on the solution treatment temperature. A preferred amount is 22% Fe and a preferred solution treatment temperature is 1140-1170°C.
3. Samarium and zirconium must be regarded as "effective" amounts to allow for the presence of oxygen and carbon respectively, as taught in our co-pending application.
4. Sufficient samarium must be present to ensure that when the 1-5 Sm-Co phase network is formed within the 2-17 Sm-Co matrix in the aging process, the 1-5 Sm-Co phase network is continuous. This is necessary for good coercivity and loop squareness (H_{K}). A preferred amount of effective samarium is 23.0%.
5. The effective zirconium present has a critical effect on the precise temperature at which the above aging transformation takes place. A preferred amount of effective zirconium is 1.4 to 2.0% with aging treatments of 845±5°C-815±5°C respectively for 20 hours.
6. The copper present influences beneficially the final transformation of regions of the 1-5 Sm-Co phase network into coherent regions of 2-17 Sm-Co phase during the controlled cooling from the primary aging temperature in the range of 800-860°C to the secondary aging temperature and then holding at that temperature. The coherent regions of 2-17 Sm-Co phase distort or strain the 1-5 Sm-Co phase network which results in high coercivity. A preferred amount of copper is 4.6%. A preferred cooling rate is 2°C/min from 860°C to 600°C and 1°C/min from 600°C to 410°C. A preferred secondary aging temperature is 410°C. A preferred holding time at 410°C is 10 hours.
7. A stated earlier, both zirconium and copper levels must be controlled to permit the iron level to be optimized whilst still permitting all the alloying elements to go into uniform solid solution in the solution treatment step.

### References

⁽¹⁾ Wallace, W. E., "Rare Earth Intermetallics", Academic Press, New York, 1973.
⁽²⁾ Tokunaga, M., Hagi, C. and Murayama, H., "Permanent Magnet Alloy", U.S. Patent No. 4,172,717, October 30, 1979.
⁽³⁾ Yoneyama, T., Tomizawa, S., Hori, T. and Ojima, T., "R₂CO₁₇ Rare Type Earth Cobalt Permanent Magnet Material and Process for Producing the Same", U.S. Patent No. 4,213,803, July 22, 1980.
⁽⁴⁾ Imaizumi, N. and Wakana, K., "Rare Earth-Cobalt System Permanent Magnetic Alloys and Method of Preparing Same", U.S. Patent No. 4,221,613, September 9, 1980.
⁽⁵⁾ Tawara, Y., Chino, T. and Ohasi, K., "Rare Earth Metal-Containing Alloys for Permanent Magnets", U.S. Patent No. 4,375,996, March 8, 1983.
⁽⁶⁾ Semones, B. C., "High Energy Density Rare Earth-Cobalt Magnets and D.C. Servo Motors: A Valuable Union", Sixth International Workshop on Rare Earth-Cobalt Permanent Magnets, Baden, Vienna, Austria, 1982.
⁽⁷⁾ Hadjipanayis, G. C., "Microstructure and Magnetic Domain Structure of 2:17 Permanent Magnets", Sixth International Workshop on Rare Earth-Cobalt Permanent Magnets, Baden, Vienna, Austria, 1982.
⁽⁸⁾ Yoneyama, T., Tomizawa, S., Hori, T. and Ojima, T., "New Type Rare Earth-Cobalt Magnets Based on Sm,(Co, Cu, Fe, M)₁₇", Third International Workshop on Rare Earth-Cobalt Permanent Magnets, La Jolla, California, 1978.
⁽⁹⁾ Yoneyama, T., Fukuno, A. and Ojima, T., "Sm₂(Co, Cu, Fe, Zr)₁₇ Magnets Having High ᵢH_{c} and (BH)ₘₐₓ'', Third International Conference on Ferrites, Kyoto, Japan, 1980.
⁽¹⁰⁾ Hadjipanayis, G. C., Hazelton, R. C., Wollins, S. H., Wysiekierski, A. and Lawless, K. R., "The Effect of Heat Treatment on the Microstructure and Magnetic Properties of a Sm(Co, Fe, Cu, Zr)₇.₂ Magnet", Sixth International Workshop on Rare Earth-Cobalt Permanent Magnets, Baden, Vienna, Austria, 1982.
⁽¹¹⁾ Fidler, J. and Skalicky, P., "Domain Wall Pinning in REPM", Proceedings of the Sixth International Workshop on Rare Earth Cobalt Permanent Magnets, Vienna, Austria, September 1982.
(¹²) Kronmuller, N., "Nucleation and Propagation of Reversed Domains in RE-Co-Magnets", Proceedings of the Sixth International Workshop on Rare Earth Cobalt Permanent Magnets, Vienna, Austria, September 1982.
(¹³) Rabenberg, L., Mishra, R. K. and Thomas, G., "Development of the Cellular Microstructure in SₘCO_{7.4} Type Magnets", Proceedings of the Sixth International Workshop on Rare Earth Cobalt Permanent Magnets, Vienna, Austria, September 1982.
⁽¹⁴⁾ Ray, A. E., "Metallurgical Behaviour of Sm(Co, Fe, Cu, Zr), Alloys", J. Appl. Phys. 55 (6), 15 March 1984.

## Claims

1. An Sm₂Co₁₇ alloy suitable for use in the manufacture of permanent magnets of high energy product and high coercivity, said alloy containing samarium, iron, copper, zirconium, cobalt and incidental amounts of carbon and oxygen, characterised in that said alloy consists of, on a weight basis and apart from impurities:
(a) an amount of samarium that is equal to from 22.5 to 23.5% of the alloy plus an additional percentage that is equal to from 4 to 9 times the amount of oxygen;
(b) from 20.0 to 25.0% Fe;
(c) from 3.0 to 5.0% Cu;
(d) an amount of zirconium that is equal to from 1.4 to 2.0% of the alloy plus an additional percentage that is equal to from 5 to 10 times-the amount of carbon;
(e) not more than 0.6% oxygen;
(f) not more than 0.1% carbon; and
(g) balance cobalt; said alloy having a crystallographic structure comprising cells of 2-17 Sm-Co rhombohedral phase surrounded by a continuous network of the 1-5 Sm-Co hexagonal phase, such structure being obtainable by:
(i) sintering an alloy of the required chemical composition at a temperature at which the alloy consists in the form of a solid/liquids mixture, the solid phase consisting essentially of solid grains of 2-17 Sm-Co and the surrounding liquid phase comprising a CuSm phase and a Zr-rich phase;
(ii) cooling the sintered alloy slowly to a solid solution treatment temperature marginally below the solid+liquid/solid transformation temperature of the alloy, thereby to form a homogeneous solid solution of said CuSm and Zr-rich phases in the 2-17 Sm-Co phase;
(iii) holding the alloy at said solid solution treatment temperature to promote the formation of said solid solution;
(iv) quenching the alloy from said solution treatment temperature to room temperature;
(v) reheating the alloy to a first aging temperature at which the solid solution transforms into a structure comprising a network of the 1-5 Sm-Co phase within a 2-17 Sm-Co matrix;
(vi) cooling the alloy slowly to a second aging temperature to cause regions of the 2-17 Sm-Co phase to nucleate coherently within the 1-5 Sm-Co phase network and thereby to create lattice strain therein; and
(vii) recooling the alloy to room temperature.

2. An alloy according to claim 1, characterised in that the composition of the alloy is as follows:
(a) 23.0% Sm plus an additional percentage that is equal to from 4 to 9 times the amount of oxygen;
(b) 22.0% Fe;
(c) 4.6% Cu;
(d) 1.7% Zr plus an additional percentage that is equal to from 5 to 10 times the amount of carbon;
(e) not more than 0.6% oxygen;
(f) not more than 0.1% carbon; and
(g) the balance cobalt.

3. An alloy according to claim 1 or 2, wherein the additional amount of Sm is 6.265 times the oxygen content of the alloy.

4. An alloy according to claim 1, 2 or 3, wherein the additional amount of Zr is 7.595 times the carbon content of the alloy.

5. An S_{M2}C_{O17} alloy, being an alloy as defined in claim 1 and obtained in the same way, but modified in that, instead of said 22.5 to 23.5% samarium plus said additional amount, some of that samarium is replaced on an atom-for-atom basis by praseodymium.

6. An alloy according to claim 5 which contains 20% Sm and 2.5% Pr plus said additional amount of samarium equal to 4 to 9 times the oxygen content of the alloy.

7. An alloy according to claim 5 or 6, wherein the additional amount of Sm is 5.871 times the oxygen content.

8. An Sm₂Co₁₇ alloy, being an alloy as defined in claim 1 and obtained in the same way, but modified in that at least some of the zirconium is replaced on an atom-for-atom basis by hafnium.

9. An alloy according to claim 8, wherein the zirconium is completely replaced by hafnium, the amount of hafnium in the alloy being equal to 2.7 to 4.0% plus an additional amount which is in the range of from 10 to 20 times the carbon content of the alloy.

10. An alloy according to claim 9, wherein the additional amount of Hf is 14.862 times the carbon content of the alloy.

11. The use of an alloy as claimed in any one of the preceding claims as a permanent magnet.

12. A process for producing an Sm₂Co,ᵣ alloy as claimed in any one of claims 1-4, characterised in that the process comprises:-
(i) forming a preliminary alloy of the required composition;
(ii) sintering the preliminary alloy at a temperature at which the alloy consists in the form of a solid/liquids mixture, the solid phase consisting essentially of solid grains of 2-17 Sm-Co, and the surrounding liquid phase comprising a CuSm phase and a Zr-rich phase;
(iii) cooling the sintered alloy slowly to a solid solution treatment temperature marginally below the solid+liquid/solid transformation temperature of the alloy, thereby to form a homogeneous solid solution of said CuSm and Zr-rich phases in the 2-17 Sm-Co phase;
(iv) holding the alloy at said solid solution treatment temperature to promote the formation of said solid solution;
(v) quenching the alloy from said solution treatment temperature to room temperature;
(vi) reheating the alloy to a first aging temperature at which the solid solution transforms into a structure comprising a network of the 1-5 Sm-Co phase within a 2-17 Sm-Co matrix;
(vii) cooling the alloy slowly to a second aging temperature to cause regions of the 2-17 Sm-Co phase to nucleate coherently within the 1-5 Sm-Co phase network and thereby to create lattice strain therein; and
(viii) recooling the alloy to room temperature.

13. A process for producing an Sm₂Co₁₇ alloy as claimed in claim 5, 6 or 7, characterised in that the process comprises:-
(i) forming a preliminary alloy of the required composition;
(ii) sintering the preliminary alloy at a temperature at which the alloy consists in the form of a solid/liquids mixture, the solid phase consisting essentially of solid grains of 2-17 Sm-Co, and the surrounding liquid phase comprising a CuSm phase and a Zr-rich phase;
(iii) cooling the sintered alloy slowly to a solid solution treatment temperature marginally below the solid+liquid/solid transformation temperature of the alloy, thereby to form a homogeneous solid solution of said CuSm and Zr-rich phases in the 2-17 Sm-Co phase;
(iv) holding the alloy at said solid solution treatment temperature to promote the formation of said solid solution;
(v) quenching the alloy from said solution treatment temperature to room temperature;
(vi) reheating the alloy to a first aging temperature at which the solid solution transforms into a structure comprising a network of the 1-5 Sm-Co phase within a 2-17 Sm-Co matrix;
(vii) cooling the alloy slowly to a second aging temperature to cause regions of the 2-17 Sm-Co phase to nucleate coherently within the 1-5 Sm-Co phase network and thereby to create lattice strain therein; and
(viii) recooling the alloy to room temperature.

14. A process for producing an Sm2Co" alloy as claimed in claim 8, 9 or 10, characterised in that the process comprises:-
(i) forming a preliminary alloy of the required composition;
(ii) sintering the preliminary alloy at a temperature at which the alloy consists in the form of a solid/liquids mixture, the solid phase consisting essentially of solid grains of 2-17 Sm-Co, and the surrounding liquid phase comprising a CuSm phase and a Zr-rich phase;
(iii) cooling the sintered alloy slowly to a solid solution treatment temperature marginally below the solid+liquid/solid transformation temperature of the alloy, thereby to form a homogeneous solid solution of said CuSm and Zr-rich phases in the 2-17 Sm-Co phase;
(iv) holding the alloy at said solid solution treatment temperature to promote the formation of said solid solution;
(v) quenching the alloy from said solution treatment temperature to room temperature;
(vi) reheating the alloy to a first aging temperature at which the solid solution transforms into a structure comprising a network of the 1-5 Sm-Co phase within a 2-17 Sm-Co matrix;
(vii) cooling the alloy slowly to a second aging temperature to cause regions of the 2-17 Sm-Co phase to nucleate coherently within the 1-5 Sm-Co phase network and thereby to create lattice strain therein; and
(viii) recooling the alloy to room temperature.

## Patentansprüche

1. Sm₂Co₁₇-Legierung, die zur Verwendung bei der Herstellung von Dauermagneten mit hohem Energieprodukt und hoher Koerzitivkraft geeignet ist sowie Samarium, Eisen, Kupfer, Zirkonium, Kobalt und zufällige Mengen an Kohlenstoff sowie Sauerstoff enthält, dadurch gekennzeichnet, daß die Legierung auf Gewichtsbasis und abgesehen von Verunreinigungen besteht aus:
(a) einer Menge an Samarium gleich 22,5 bis 23,5% der Legierung plus einem zusätzlichen Prozentsatz, der gleich dem 4-9-fachen der Menge an Sauerstoff ist;
(b) 20,0 bis 25,0% Fe;
(c) 3,0 bis 5,0% Cu;
(d) einer Menge an Zirkonium gleich 1,4 bis 2,0% der Legierung plus einem zusätzlichen Prozentsatz, der dem 5-10-fachen der Menge an Kohlenstoff gleich ist;
(e) nicht mehr als 0,6% Sauerstoff;
(f) nicht mehr als 0,1% Kohlenstoff; und
(g) Kobalt als Rest; wobei diese Legierung eine kristallographische Struktur hat, die Zellen einer 2-17 Sm-Corhomboedrischen Phase, umgeben von einem kontinuierlichen Netzwerk der 1-5 Sm-Co-hexagonalen Phase aufweist, und diese Struktur erzielbar ist durch:
(i) Sintern einer Legierung mit der geforderten chemischen Zusammensetzung bei einer Temperatur, bei welcher die Legierung in Form einer Fest/Flüssig-Mischung vorliegt, wobei die feste Phase im wesentlichen aus Festkörnern von 2-17 Sm-Co besteht und die umgebende flüssige Phase eine Cu-Sm-Phase sowie eine Zr-reiche Phase umfasst;
(ii) langsames Abkühlen der gesinterten Legierung knapp unter die Fest+Flüssig/Fest-Umwandlungstemperatur der Legierung, um dadurch einen homogenen Mischkristall der CuSm- und Zr-reichen Phasen in der 2-17 Sm-Co-Phase zu bilden;
(iii) Halten der Legierung auf der Mischkristall-Behandlungstemperatur, um die Bildung des Mischkristalls zu fördern;
(iv) rasches Abkühlen der Legierung von der Mischkristall-Behandlungstemperatur auf Raumtemperatur;
(v) erneutes Erhitzen der Legierung auf eine erste Alterungstemperatur, bei der sich der Mischkristall in eine ein Netzwerk der 1-5 Sm-Co-Phase innerhalb einer 2-17 Sm-Co-Matrix umfassende Struktur umwandelt;
(vi) langsames Abkühlen der Legierung auf eine zweite Alterungstemperatur, um Bereiche der 2-17 Sm-Co-Phase zur kohärenten Kernbildung innerhalb des 1-5 Sm-Co-Phasennetzwerks zu veranlassen und dadurch darin eine Gitterspannung zu erzeugen; und
(vii) erneutes Abkühlen der Legierung auf Raumtemperatur.

2. Legierung nach Anspruch 1, dadurch gekennzeichnet, daß die Legierung die folgende Zusammensetzung hat:
(a) 23,0% Sm plus einen zusätzlichen Prozentsatz, der der 4-9fachen Menge an Sauerstoff entspricht;
(b) 22,0% Fe;
(c) 4,6% Cu;
(d) 1,7% Zr plus einen zusätzlichen Prozentsatz, der der 5-10fachen Menge an Kohlenstoff gleich ist;
(e) nicht mehr als 0,6% Sauerstoff;
(f) nicht mehr als 0,1% Kohlenstoff; und
(g) Kobalt als Rest.

3. Legierung nach Anspruch 1 oder 2, dadurch gekennzeichnet, daß die zusätzliche Menge an Sm das 6,265fache des Sauerstoffgehalts der Legierung ist.

4. Legierung nach Anspruch 1, oder 3, dadurch gekennzeichnet, daß die zusätzliche Menge an Zr das 7,595fache des Kohlenstoffgehalts der Legierung ist.

5. Sm₂Co₁₇-Legierung, die eine im Anspruch 1 definierte sowie in gleichartiger Weise erhaltene, jedoch insoweit modifizierte Legierung ist, als anstelle der 22,5 bis 23,5% Samarium plus der genannten zusätzlichen Menge ein Teil des Samariums auf einer Atom-für-Atom-Basis durch Praseodym ersetzt ist.

6. Legierung nach Anspruch 5, dadurch gekennzeichnet, daß sie 20% Sm und 2,5% Pr plus der zusätzlichen Menge an Samarium gleich dem 4-9fachen des Sauerstoffgehalts der Legierung enthält.

7. Legierung nach Anspruch 5 oder 6, dadurch gekennzeichnet, daß die zusätzliche Menge an Sm das 5,871fache des Sauerstoffgehalts ist.

8. Sm2Co17-Legierung, die eine im Anspruch 1 definierte sowie in gleichartiger Weise erhaltene, jedoch insoweit modifizierte Legierung ist, als wenigstens ein Teil des Zirkoniums auf einer Atom-für-Atom-Basis durch Hafnium ersetzt ist.

9. Legierung nach Anspruch 8, dadurch gekennzeichnet, daß das Zirkonium vollständig durch Hafnium ersetzt ist, wobei die Menge an Hafnium in der Legierung gleich 2,7 bis 4,0% plus einer zusätzlichen Menge, die im Bereich des 1020fachen des Kohlenstoffgehalts der Legierung liegt, beträgt.

10. Legierung nach Anspruch 9, dadurch gekennzeichnet, daß die zusätzliche Menge an Hf das 14,862fache des Kohlenstoffgehalts der Legierung ist.

11. Verwendung einer Legierung nach einem der vorhergehenden Ansprüche als ein Dauermagnet.

12. Verfahren zur Herstellung einer Sm2Co17-Legierung, wie sie in einem der Ansprüche 1-4 definiert ist, dadurch gekennzeichnet, daß das Verfahren umfaßt:
(i) Ausbilden einer Vorlegierung der geforderten Zusammensetzung;
(ii) Sintern der Vorlegierung bei einer Temperatur, bei der die Legierung in Form einer Fest/Flüssig-Mischung vorliegt, wobei die feste Phase im wesentlichen aus Festkörnern von 2-17 Sm-Co besteht und die umgebende flüssige Phase eine CuSm-Phase sowie eine Zr-reiche Phase umfaßt;
(iii) langsames Abkühlen der Legierung auf eine Misch-kristall-Behandlungstemperatur knapp unter der Fest+Flüssig/Fest-Umwandlungstemperatur der Legierung, um dadurch einen homogenen Mischkristall der CuSm- und Zr-reichen Phasen in der 2-17 Sm-Co-Phase zu bilden;
(iv) Halten der Legierung auf der Mischkristall-Behandlungstemperatur, um die Bildung des Mischkristalls zu fördern;
(v) rasches Abkühlen der Legierung von der Mischkristall-Behandlungstemperatur auf Raumtemperatur;
(vi) erneutes Erhitzen der Legierung auf eine erste Alterungstemperatur, bei der sich der Mischkristall in eine ein Netzwerk der 1-5 Sm-Co-Phase innerhalb einer 2-17 Sm-Co-Matrix umfassende Struktur umwandelt;
(vii) langsames Abkühlen der Legierung auf eine zweite Alterungstemperatur, um Bereiche der 2-17 Sm-Co-Phase zur kohärenten Kernbildung innerhalb des 1-5 Sm-Co-Phasennetzwerks zu veranlassen und dadurch darin eine Gitterspannung zu erzeugen; und
(viii) erneutes Abkühlen der Legierung auf Raumtemperatur.

13. Verfahren zur Herstellung einer Sm₂CO₁₇-Legierung, wie sie in Anspruch 5, 6 oder 7 definiert ist, dadurch gekennzeichnet, daß das Verfahren umfaßt:
(i) Ausbilden einer Vorlegierung der geforderten Zusammensetzung;
(ii) Sintern der Vorlegierung bei einer Temperatur, bei der die Legierung in Form einer Fest/Flüssig-Mischung vorliegt, wobei die feste Phase im wesentlichen aus Festkörnern von 2-17 Sm-Co besteht und die umgebende flüssige Phase eine CuSm-Phase sowie eine Zr-reiche Phase umfaßt;
(iii) langsames Abkühlen der Legierung auf eine Mischkristall-Behandlungstemperatur knapp unter der Fest+Flüssig/Fest-Umwandlungstemperatur der Legierung, um dadurch einen homogenen Mischkristall der CuSm- und Zr-reichen Phasen in der 2-17 Sm-Co-Phase zu bilden;
(iv) Halten der Legierung auf der Mischkristall-Behandlungstemperatur, um die Bildung des Mischkristalls zu fördern;
(v) rasches Abkühlen der Legierung von der Mischkristall-Behandlungstemperatur auf Raumtemperatur;
(vi) erneutes Erhitzen der Legierung auf eine erste Alterungstemperatur, bei der sich der Mischkristall in eine ein Netzwerk der 1-5 Sm-Co-Phase innerhalb einer 2-17 Sm-Co-Matrix umfassende Struktur umwandelt;
(vii) langsames Abkühlen der Legierung auf eine zweite Alterungstemperatur, um Bereiche der 2-17 Sm-Co-Phase zur kohärenten Kernbildung innerhalb des 1-5 Sm-Co-Phasennetzwerks zu veranlassen und dadurch darin eine Gitterspannung zu erzeugen; und
(viii) erneutes Abkühlen der Legierung auf Raumtemperatur.

14. Verfahren zur Herstellung einer Sm₂Co₁₇-Legierung, wie sie in Anspruch 8, 9 oder 10 definiert ist, dadurch gekennzeichnet, daß das Verfahren umfaßt:
(i) Ausbilden einer Vorlegierung der geforderten Zusammensetzung;
(ii) Sintern der Vorlegierung bei einer Temperatur, bei der die Legierung in Form einer Fest/Flüssig-Mischung vorliegt, wobei die feste Phase im wesentlichen aus Festkörnern von 2-17 Sm-Co besteht und die umgebende flüssige Phase eine CuSm-Phase sowie eine Zr-reiche Phase umfaßt;
(iii) langsames Abkühlen der Legierung auf eine Mischkristall-Behandlungstemperatur knapp unter der Fest+Flüssig/Fest-Umwandlungstemperatur der Legierung, um dadurch einen homogenen Mischkristall der CuSm- und Zr-reichen Phasen in der 2-17 Sm-Co-Phase zu bilden;
(iv) Halten der Legierung auf der Mischkristall-Behandlungstemperatur, um die Bildung des Mischkristalls zu fördern;
(v) rasches Abkühlen der Legierung von der Mischkristall-Behandlungstemperatur auf Raumtemperatur;
(vi) Erneutes Erhitzen der Legierung auf eine erste Alterungstemperatur, bei der sich der Mischkristall in eine ein Netzwerk der 1-5 Sm-Co-Phase innerhalb einer 2-17 Sm-Co-Matrix umfassende Struktur umwandelt;
(vii) langsames Abkühlen der Legierung auf eine zweite Alterungstemperatur, um Bereiche der 2-17 Sm-Co-Phase zur kohärenten Kernbildung innerhalb des 1-5 Sm-Co-Phasennetzwerks zu veranlassen. und dadurch darin eine Gitterspannung zu erzeugen; und
(viii) erneutes Abkühlen der Legierung auf Raumtemperatur.

## Revendications

1. Un alliage de Sm2Co" utilisable dans la fabrication des aimants permanents d'énergie élevée et de coercitivité élevée, ledit alliage contenant du samarium, du fer, du cuivre, du zirconium, du cobalt et des quantités accidentelles de carbone et d'oxygène, caractérisé en ce que ledit alliage consiste, sur une base pondérale et abstraction faite des impuretés, en:
(a) une quantité de samarium qui est égale à 22,5 à 23,5% de l'alliage plus un pourcentage additionnel qui est égal à 4 à 9 fois la quantité d'oxygène;
(b) de 20,0 à 25,0% de Fe;
(c) de 3,0 à 5,0% de Cu;
(d) une quantité de zirconium qui est égale à 1,4 à 2,0% de l'alliage plus un pourcentage additionnel qui est égal à 5 à 10 fois la quantité de carbone;
(e) au plus 0,6% d'oxygène;
(f) au plus 0,1% de carbone; et
(g) le restant étant du cobalt; ledit alliage ayant une structure cristallographique comprenant des cellules de phase rhomboédrique 2-17 Sm-Co entourées par un réseau continu de phase hexagonale 1-5 Sm-Co, une telle structure étant procurable par:
(i) frittage d'un alliage de la composition chimique requise à une température à laquelle l'alliage consiste en la forme d'un mélange de solide/liquides, la phase solide consistant essentiellement en grains solides de 2-17 Sm-Co, et la phase liquide entourante comprenant une phase de CuSm et une phase riche en Zr;
(ii) refroidissement de l'alliage fritté lentement à une température de traitement de solution solide de façon marginale inférieure à la température de transformation solide+liquide/solide de l'alliage, pour former une solution solide homogène de ladite phase de CuSm et de ladite phase riche en Zr dans la phase 2-17 Sm-Co;
(iii) maintien de l'alliage à ladite température de traitement de solution solide pour favoriser la formation de ladite solution solide;
(iv) trempe de l'alliage depuis ladite température de traitement de solution à la température ambiante;
(v) réchauffage de l'alliage à une première température de vieillissement à laquelle la solution solide se transforme en une structure comprenant un réseau de la phase de 1-5 Sm-Co à l'intérieur d'une matrice de 2-17 Sm-Co;
(vi) refroidissement de l'alliage lentement à une seconde température de vieillissement pour provoquer la nucléation cohérente des régions de la phase de 2-17 Sm-Co à l'intérieur du réseau de phase de 1-5 Sm-Co et pour y créer ainsi une déformation du réseau; et
(vii) nouveau refroidissement de l'alliage à la température ambiante.

2. Un alliage selon la revendication 1, caractérisé en ce que la composition de l'alliage est la suivante:
(a) 23,0% de Sm plus un pourcentage additionnel qui est égal à 4 à 9 fois la quantité d'oxygène;
(b) 22,0% de Fe;
(c) 4,6% de Cu;
(d) 1,7% de Zr plus un pourcentage additionnel qui est égal à 5 à 10 fois la quantité de carbone;
(e) au plus 0,6% d'oxygène;
(f) au plus 0,1% de carbone; et
(g) le restant étant du cobalt.

3. Un alliage selon la revendication 1 ou 2, selon lequel la quantité additionnelle de Sm est de 6,265 fois la teneur en oxygène de l'alliage.

4. Un alliage selon la revendication 1, 2 ou 3, selon lequel la quantité additionnelle de Zr est de 7,595 fois la teneur en carbone de l'alliage.

5. Un alliage de S_{M2}C_{O17}, qui est un alliage tel que défini dans la revendication 1 et obtenu de la même façon, mais modifié par le fait que, au lieu de ladite quantité de 22,5 à 23,5% de samarium plus ladite quantité additionnelle, une certaine quantité de samarium est remplacée par le praséodyme sur la base d'un atome par atome.

6. Un alliage selon la revendication 5 qui contient 20% de Sm et de 2,5% de Pr plus ladite quantité additionnelle de samarium égale à 4 à 9 fois la teneur en oxygène de l'alliage.

7. Un alliage selon la revendication 5 ou 6, selon lequel la quantité additionnelle de Sm est de 5,871 fois la teneur en oxygène.

8. Un alliage de Sm₂C₀₁₇ qui est un alliage tel que défini dans la revendication 1 et obtenu de la même façon, mais modifié par le fait qu'au moins une certaine quantité de zirconium est remplacée par du hafnium sur la base d'un atome par atome.

9. Un alliage selon la revendication 8, selon lequel le zirconium est complètement remplacé par le hafnium, la quantité de hafnium dans l'alliage étant égale à 2,7 à 4,0% plus une quantité additionnelle qui est dans l'intervalle de 10 à 20 fois la teneur en carbone de l'alliage.

10. Un alliage selon la revendication 9, selon lequel la quantité additionnelle de Hf est de 14,862 fois la teneur en carbone de l'alliage.

11. Utilisation d'un alliage selon l'une quelconque des revendications précédentes comme aimant permanent.

12. Un procédé de production d'un alliage de Sm2Co" selon l'une quelconque des revendications 1-4, caractérisé en ce que le procédé comprend:
(i) la formation d'un alliage préliminaire ayant la composition requise;
(ii) le frittage de l'alliage préliminaire à une température à laquelle l'alliage consiste en la forme d'un mélange de solide/liquides, la phase solide consistant essentiellement en grains solides de 2-17 Sm-Co, et la phase liquide entourante comprenant une phase de CuSm et une phase riche en Zr;
(iii) le refroidissement de l'alliage fritté lentement à une température de traitement de solution solide de façon marginale inférieure à la température de transformation de solide+liquide/solide de l'alliage, pour former une solution solide homogène de ladite phase de CuSm et de ladite phase riche en Zr dans la phase de 2-17 Sm-Co;
(iv) le maintien de l'alliage à ladite température de traitement de solution solide pour favoriser la formation de ladite solution solide;
(v) la trempe de l'alliage depuis ladite température de traitement de solution à la température ambiante;
(vi) le réchauffage de l'alliage à une première température de vieillissement à laquelle ladite solution solide se transforme en une structure comprenant un réseau de la phase de 1-5 Sm-Co à l'intérieur d'une matrice de 2-17 Sm-Co;
(vii) le refroidissement de l'alliage lentement à une seconde température de vieillissement pour provoquer la nucléation cohérente des régions de la phase de 2-17 Sm-Co à l'intérieur du réseau de la phase 1-5 Sm-Co et pour y créer une déformation du réseau; et
(viii) un nouveau refroidissement de l'alliage à la température ambiante.

13. Un procédé de production d'un alliage de Sm₂C₀₁₇ selon la revendication 5, ou 7, caractérisé en ce que le procédé comprend:
(i) la formation d'un alliage préliminaire ayant la composition requise;
(ii) le frittage de l'alliage préliminaire à une température à laquelle l'alliage consiste en la forme d'un mélange de solide/liquides, la phase solide consistant essentiellement en grains solides de 2-17 Sm-Co, et la phase liquide entourante comprenant une phase de CuSm et une phase riche en Zr;
(iii) le refroidissement de l'alliage fritté lentement à une température de traitement de solution solide de façon marginale inférieure à la température de transformation de solide+liquide/solide de l'alliage, pour former une solution solide homogène de ladite phase de CuSm et de ladite phase riche en Zr dans la phase de 2-17 Sm-Co;
(iv) le maintien de l'alliage à ladite température de traitement de solution solide pour favoriser la formation de ladite solution solide;
(v) la trempe de l'alliage depuis ladite température de traitement en solution à la température ambiante;
(vi) le réchauffage de l'alliage à une première température de vieillissement à laquelle ladite solution solide se transforme en une structure comprenant un réseau de la phase de 1-5 Sm-Co à l'intérieur d'une matrice de 2-17 Sm-Co;
(vii) le refroidissement de l'alliage lentement à une seconde température de vieillissement pour provoquer la nucléation cohérente des régions de la phase de 2-17 Sm-Co à l'intérieur du réseau de la phase de 1-5 Sm-Co et pour y créer une déformation du réseau; et
(viii) un nouveau refroidissement de l'alliage à la température ambiante.

14. Un procédé de production d'un alliage de Sm₂Co₁₇ selon la revendication 8, ou 10, caractérisé en ce que le procédé comprend:
(i) la formation d'un alliage préliminaire ayant la composition requise;
(ii) le frittage de l'alliage préliminaire à une température à laquelle l'alliage consiste en la forme d'un mélange de solide/liquides, la phase solide consistant essentiellement en grains solides de 2-17 Sm-Co, et la phase liquide entourante comprenant une phase de CuSm et une phase riche en Zr;
(iii) le refroidissement de l'alliage fritté lentement à une température de traitement de solution solide de façon marginale inférieure à la température de transformation de solide+liquide/solide de l'alliage, pour former une solution solide homogène de ladite phase de CuSm et de ladite phase riche en Zr dans la phase de 2-17 Sm-Co;
(iv) le maintien de l'alliage à ladite température de traitement de solution solide pour favoriser la formation de ladite solution solide;
(v) la trempe de l'alliage depuis ladite température de traitement en solution à la température ambiante;
(vi) le réchauffage de l'alliage à une première température de vieillissement à laquelle ladite solution solide se transforme en une structure comprenant un réseau de la phase de 1-5 Sm-Co à l'intérieur d'une matrice de 2-17 Sm-Co;
(vii) le refroidissement de l'alliage lentement à une seconde température de vieillissement pour provoquer la nucléation cohérente des régions de la phase de 2-17 Sm-Co à l'intérieur du réseau de la phase de 1-5 Sm-Co et pour y créer une déformation du réseau; et
(viii) un nouveau refroidissement de l'alliage à la température ambiante.
